

# UNITED STATES PATENT OFFICE.

HERMANN SCHÖNEWEG, OF DUDWEILER, NEAR SAARBRÜCKEN, PRUSSIA,  
GERMANY.

## EXPLOSIVE.

SPECIFICATION forming part of Letters Patent No. 371,376, dated October 11, 1887.

Application filed July 6, 1887. Serial No. 240,425. (No specimens.)

*To all whom it may concern:*

Be it known that I, HERMANN SCHÖNEWEG, a subject of the King of Prussia, German Emperor, and a resident of Dudweiler, near Saarbrücken, in the Kingdom of Prussia, German Empire, have invented certain new and useful Improvements in Explosive Materials, of which the following is a specification.

The object of the improvements described hereinafter is to smother the ignition-flames of explosives when discharged and to render them harmless. When explosives are used in coal-mines for blasting purposes, their ignition-flames have often proved the cause of disastrous explosions of black-damp or coal-dust.

These improvements consist in adding oxalic acid or one of the oxalates to the usual explosive substances. The effect produced by this addition of oxalic acid or of an oxalate to the well known explosives is of a two-fold nature: First of all, the ignition-flames are smothered when the explosion takes place, and, secondly, the compound acquires greater explosive power by this addition, for the oxalic acid or the oxalate is decomposed when explosion takes place and greatly augments the effect of the blasting. In addition to this, the oxalic acid or the oxalate prevents the actual explosive substances from decomposition, and consequently makes the explosives much more durable.

The oxalic acid or the oxalate is incorporated with the explosive substances in the following way: Nitrate of ammonia is first dissolved, by putting five per cent. of water to it. Forty per cent., by weight, of oxalic acid or of an oxalate—for instance, oxalate of ammonium—is then added to one hundred per cent., by weight, of the dissolved nitrate of ammonia. When mixed, the compound is dried at a temperature of 60° to 80° Celsius till it loses no longer in weight. By this means a perfectly-anhydrous compound of an amorphous consistency is obtained. This amorphous compound is then added to the explosive. If the explosives the ignition-flames of which have to be smothered by the addition of oxalic acid or of an oxalate con-

sist in liquid nitrated carburets of hydrogen, 50 (for instance, nitro-benzol, nitro-toluol, or nitro-naphthaline,) then ten per cent., by weight, of the amorphous compound just described is added to ninety per cent., by weight, of the original explosive. If the original explosives consist in solid nitrated carburets of hydrogen, or if they be of a gelatinous consistency, like the well-known Nobel's blast-gelatine, or if they be the well-known guhr-dynamite, up to twenty per cent. of the amorphous compound described above may be added to eighty per cent. of the explosives.

For the sake of greater clearness, two compounds which are well adapted for making 65 pasty and granulated explosives will be now described.

First. Pasty explosives are obtained by mixing eighty per cent. of nitro-benzol or nitro-toluol with twenty per cent. of dinitro-benzol, dinitro-naphthaline, or trinitro-naphthaline. Thirty per cent. of nitrated cellulose (gun-cotton or collodion gun-cotton) is dissolved in this mixture, and the result is a gelatinous compound, which is incorporated 75 with twenty per cent. of oxalic acid or of one of the oxalates, or with twenty per cent. of the compound described above.

Second. Granulated explosives are obtained by mixing eighty per cent. of dinitro-benzol, or dinitro-naphthaline, or trinitro-naphthaline with twenty per cent. of nitro-benzol or nitro toluel. In these explosives, which form an amorphous powder, thirty per cent. of nitrated cellulose (gun-cotton or collodion gun-cotton) is then dissolved by heating the powder up to 70° Celsius. When the mixture is cooled, an amorphous granulated substance is obtained, with which twenty per cent. of oxalic acid or oxalates, or of the above-90 described compound, is mixed.

All the well-known oxalates may be used for this purpose. All these oxalates may be used in the manner described above. The most important of them are potassic hydric 95 oxalate, oxalate of ammonium, ammonium hydric oxalate, likewise oxalate of potassic ammonium and oxalate of sodic ammonium.

Having fully described my invention, what I claim, and desire to secure by Letters Patent of the United States, is—

5 An explosive compound consisting in nitrated carburets of hydrogen and nitrated celulose with an oxalate or oxalic acid, for the purpose specified.

In witness whereof I have hereunto set my hand in presence of two witnesses.

HERMANN SCHÖNEWEG.

Witnesses:

A. MÜHLNER,  
B. ROI.